

Patented Nov. 10, 1936

2,060,563

# UNITED STATES PATENT OFFICE

2,060,563

## AZO DYESTUFFS CONTAINING CHROMIUM AND PROCESS OF PREPARING THEM

Erich Fischer, Bad Soden-on-the-Taunus, Germany, assignor to General Aniline Works, Inc., New York, N. Y., a corporation of Delaware

No Drawing. Application September 22, 1934,  
Serial No. 745,166. In Germany September 27,  
1933

10 Claims. (Cl. 260—12)

The present invention relates to new azo-dyestuffs containing chromium. It comprises the process of making these chromed dyestuffs, the chromium compounds of the dyestuffs and the material dyed with the new products.

I have found that azo-dyestuffs of valuable properties which contain chromium and yield yellow to orange tints are obtainable by treating with agents yielding chromium the pyrazolone-10 azo-dyestuffs of the following general formula:



15 wherein R stands for an aryl radical, R<sub>1</sub> stands for an aryl radical or the group —COO—alkyl, R<sub>2</sub> stands for an aryl radical containing a carboxylic acid group in one ortho-position to the azo-group and no hydroxy group in the other ortho-position to the azo-group and wherein, furthermore, at least one of the radicals R and R<sub>2</sub> must contain at least one sulfonic acid group.

20 The resultant azo-dyestuffs containing chromium have a better fastness to fulling than the dyestuffs analogous thereto which have in 3-position of the pyrazolone nucleus a carboxylic acid or alkyl group.

25 The above mentioned pyrazolone-azo-dyestuffs are obtainable by coupling diazotized ortho-amino-aryl-carboxylic acids which contain no hydroxy group in ortho-position to the amino group with 3-phenyl-5-pyrazolones or 5-pyrazolone-3-carboxylic acid alkyl esters, the components being chosen so that the dyestuffs contain at least one sulfonic acid group.

30 As diazo components which come into consideration for the preparation of the starting materials used in the present process the following may, for instance, be mentioned: 2-aminobenzene-1-carboxylic acid, 3-bromo-2-aminobenzene-1-carboxylic acid, 3,5-dichloro-2-aminobenzene-1-carboxylic acid, 5-chloro-2-aminobenzene-1-carboxylic acid, 4-aminodiphenyl-3-carboxylic acid, 4-nitro-2-aminobenzene-1-carboxylic acid, 4-sulfo-2-aminobenzene-1-carboxylic acid, 5-sulfo-2-aminobenzene-1-carboxylic acid, 3,5-disulfo-2-aminobenzene-1-carboxylic acid, 3-chloro-5-sulfo-2-aminobenzene-1-carboxylic acid, 2,3-aminonaphthoic acid or the like.

35 For the preparation of the starting dyestuffs there may be used as coupling components, for instance, the following pyrazolone compounds: 1-phenyl-3-phenyl-5-pyrazolone, 1-phenyl-5-pyrazolone-3-carboxylic acid ethyl ester, 1-(2'-chlorophenyl)-3-phenyl-5-pyrazolone, 1-(2'-chloro-5'-sulfophenyl)-3-phenyl-5-pyrazolone, 1-(3'-sulfophenyl)-3-phenyl-5-pyrazolone, 1-(2'-sulfophenyl)-3-phenyl-5-pyrazolone, 1-(4'-

methyl-2'-sulfophenyl)-3-phenyl-5-pyrazolone, 1-(4'-chloro-2'-sulfophenyl)-3-phenyl-5-pyrazolone, 1-(2',4'-dimethyl-6'-sulfophenyl)-3-phenyl-5-pyrazolone, 1-(2'-sulfophenyl)-5-pyrazolone-3-carboxylic acid ethyl ester, 1-(4'-chloro-2'-sulfophenyl)-5-pyrazolone-3-carboxylic acid methyl ester, 1-(4'-methyl-2'-sulfophenyl)-5-pyrazolone-3-carboxylic acid butyl ester, 1-(2'-methyl-6'-chloro-4'-sulfophenyl)-3-phenyl-5-pyrazolone, 1-(2'-sulfophenyl)-3-(4'-carboxyphenyl)-5-pyrazolone, 1-(2'-chloro-5'-sulfophenyl)-3-(4'-methylphenyl)-5-pyrazolone, 1-(4'-sulfo-phenyl)-5-pyrazolone-3-carboxylic acid ethyl ester, 1-(2',5'-disulfophenyl)-3-phenyl-5-pyrazolone, 1-(2',4'-disulfophenyl)-5-pyrazolone-3-carboxylic acid ethyl ester, 1-(2'-carboxy-5'-sulfophenyl)-3-phenyl-5-pyrazolone, 1-(4'-sulfo-naphthyl)-3-phenyl-5-pyrazolone,



20



25



30

1-(2'-hydroxy-3'-carboxy-5'-sulfophenyl)-3-phenyl-5-pyrazolone, 1-(2',4'-dichloro-6'-sulfophenyl)-3-phenyl-5-pyrazolone or the like.

35

The treatment of the dyestuffs with the agents yielding chromium may be effected in known manner by heating in open vessels, under reflux or under raised pressure. As agents yielding chromium there may be used, for instance chromium chloride, chromium fluoride, chromium formate or chromium acetate or other organic or inorganic chromium salts.

40

The products made in accordance with the invention are suitable, for example, for dyeing animal fibers like wool, natural and loaded silk and leather.

45

The following examples serve to illustrate the invention but they are not intended to limit it thereto, the parts being by weight:

50

(1) 544 parts of the azo-dyestuff obtainable from diazotized ortho-amino benzoic acid and 1-(2',5'-disulfophenyl)-3-phenyl-5-pyrazolone are dissolved in 5000 parts of water and heated to boiling under reflux with 300 parts of chromium formate (corresponding to 92 parts of chromium oxide) until the formation of the chromium complex is finished. The excess of chromium salt is removed by means of sodium carbonate and the filtered and neutralized solu-

60

tion is concentrated by evaporation. The powder obtained which is easily soluble in water yields according to the dyeing methods usually applied with dyestuffs containing chromium reddish-yellow even dyeings of very good fastness properties.

(2) 464 parts of the dyestuff obtainable from diazotized ortho-aminobenzoic acid and 1-(2'-sulfophenyl)-3-phenyl-5-pyrazolone are heated to boiling, under reflux, for about 30 hours in an aqueous solution with chromium fluoride corresponding to 92 parts of chromium oxide. The dyestuff containing chromium is salted out by means of sodium chloride. It yields reddish-yellow very even dyeings of very good fastness to light and good fastness to washing.

(3) By replacing in the Examples 1 and 2 the dyestuffs used therein by 661.5 parts of the pyrazolone-azo-dyestuff of the following formula:



a dyestuff of similar properties is obtained which yields shades of a more greenish hue.

30 (4) 540 parts of the dyestuff obtainable from diazotized ortho-aminobenzoic acid and 1-(2',4'-disulfophenyl)-5-pyrazolone - 3 - carboxylic acid ethyl ester are heated to boiling in an aqueous solution with chromium formate. The chromium compound of the dyestuff thus obtained yields on wool yellow dyeings of good fastness properties.

35 (5) The chromium compound of the dyestuff of the following formula:



50 which is obtainable by boiling for several hours a solution of 714.5 parts of the dyestuff in water with a chromium formate solution corresponding to 92 parts of chromium oxide is distinguished by greenish-yellow dyeings of good fastness properties.

55 (6) 544 parts of the dyestuff obtainable from diazotized 5-sulfo-2-amino-1-benzoic acid and 1 - (4'-sulfophenyl)-3-phenyl - 5 - pyrazolone are heated to boiling in a 10 per cent aqueous solution with chromium fluoride until the formation 60 of the chromium complex is finished. The dyestuff containing chromium dyes wool reddish-yellow tints of good properties.

65 (7) By replacing in the preceding examples the dyestuffs mentioned therein by 589 parts of the dyestuff of the following formula:



a dyestuff of similar properties is obtained which yields reddish-yellow tints.

(8) 464 parts of the dyestuff obtainable from diazotized ortho-aminobenzoic acid and 1-(2',4'-dimethyl-6'-sulfophenyl)-3-phenyl-5-pyrazolone are heated at 130° C. for 4 hours in an autoclave, while stirring, in an aqueous solution with chromium formate corresponding to 92 parts of chromium oxide. The chromium compound of the azo-dyestuff is completely salted out and, in the dry state, forms a yellow powder. It dyes wool yellow tints of excellent fastness to light, very good evenness and good fastness to washing.

I claim:

1. The process of preparing azo-dyestuffs containing chromium which comprises heating pyrazolone-azo-dyestuffs of the general formula:



25 wherein R stands for a radical of the benzene or naphthalene series, R1 for the group -COO-alkyl or for a radical of the benzene series, R2 represents a radical of the benzene, naphthalene or diphenyl series containing a carboxylic acid group in one o-position to the azo-group and no hydroxy group in the other o-position to the azo-group and wherein at least one of the radicals R and R2 contains at least one sulfonic acid group, with agents yielding chromium.

30 2. The process of preparing azo-dyestuffs containing chromium which comprises heating pyrazolone-azo-dyestuffs of the general formula:



45 wherein R1 stands for the group -COO-alkyl or for a radical of the benzene series, R2 represents a radical of the benzene series containing a carboxylic acid group in one o-position to the azo-group and no hydroxy group in the other o-position to the azo-group, and X1 stands for a member of the group consisting of hydrogen, methyl and chlorine and X2 for a member of the group consisting of hydrogen, methyl, chlorine and the sulfonic acid group, with agents yielding chromium.

50 3. The process of preparing an azo-dyestuff containing chromium which comprises heating a pyrazolone-azo-dyestuff of the formula:



60 with an agent yielding chromium.

5

10

15

20

25

30

35

40

45

50

55

60

65

70

75

4. The process of preparing an azo-dyestuff containing chromium which comprises heating a pyrazolone-azo-dyestuff of the formula:

5



10 15 with an agent yielding chromium.

5. The process of preparing an azo-dyestuff containing chromium which comprises heating a pyrazolone-azo-dyestuff of the formula:

20



25 30 with an agent yielding chromium.

6. The chromium compounds of the azo-dye-stuffs of the general formula:

35



wherein R stands for a radical of the benzene or naphthalene series, R<sub>1</sub> for the group —COO—alkyl or for a radical of the benzene series, R<sub>2</sub> represents a radical of the benzene, naphthalene or diphenyl series containing a carboxylic acid group in one o-position to the azo-group and no hydroxy group in the other o-position to the azo-group, wherein at least one of the radicals R and R<sub>2</sub> contains at least one sulfonic acid group, and wherein the carboxylic acid group of the radical R<sub>2</sub> standing in o-position to the azo-bridge, in combination with this azo-bridge, contains bound chromium, which products form yellow to orange powders which dye the animal fiber yellow to orange tints of good fastness properties.

7. The chromium compounds of the azo-dye-stuffs of the general formula:

55



60 65 wherein R<sub>1</sub> stands for the group —COO—alkyl or for a radical of the benzene series, R<sub>2</sub> represents a radical of the benzene series containing a carboxylic acid group in one o-position to the

azo-group and no hydroxy group in the other o-position to the azo-group, X<sub>1</sub> stands for a member of the group consisting of hydrogen, methyl and chlorine, X<sub>2</sub> for a member of the group consisting of hydrogen, methyl, chlorine and the sulfonic acid group, and wherein the carboxylic acid group of the radical R<sub>2</sub> standing in o-position to the azo-bridge, in combination with this azo-bridge, contains bound chromium, which products form yellow to orange powders which dye the animal fiber yellow to orange tints of good fastness properties.

8. The chromium compound of the azo-dye-stuff of the formula:

15



wherein the carboxylic acid group, in combination with the azo-bridge, contains bound chromium, which product forms a yellow powder dyeing the animal fiber reddish-yellow tints of very good evenness, very good fastness to light and good fastness to washing.

9. The chromium compound of the azo-dye- 30 stuff of the formula:

35



wherein the carboxylic acid group, in combination with the azo-bridge, contains bound chromium, which product forms a yellow powder dyeing the animal fiber yellow tints of very good evenness, very good fastness to light and good fastness to washing.

10. The chromium compound of the azo-dye- 50 stuff of the formula:

50



55 60 wherein the carboxylic acid group, in combination with the azo-bridge, contains bound chromium, which product forms a yellow powder dyeing the animal fiber yellow tints of very good evenness, very good fastness to light and good fastness to washing.

ERICH FISCHER.